# EUROPEAN PATENT APPLICATION

(11) **EP 1 923 228 A1**
(43) Date of publication of application: **21.05.2008**
(21) Application number: 07120223.8
(22) Date of filing: 08.11.2007
(51) Int. Cl.: B41N 1/08

(54) **Offset presensitized plate with compound support and its manufacturing process**

(30) Priority: 08.11.2006 CN 200610154602
(71) Applicant: Wenzhou Konita Printing Equipment Co., Ltd., Wenzhou, Zhejiang, 325013 (CN)
(72) Inventor: Xiangfeng, Chen, 325013 Wenzhou Zhejiang (CN)
(74) Representative: Markó, József

(57) **Abstract**

A presensitized plate with compound support includes an aluminum substrate (1) having a front side and a back side, and a sensitization imaging layer set up on the front side of the aluminum substrate, wherein the back side of the substrate (1) is covered with a membrane (2) of polymer material forming the structure of compound support.

A manufacturing process of presensitized plate with compound support according to the invention comprises deoiling and cleaning the aluminum substrate (1), conducting electrochemical corrosion and roughening for the surface of the substrate (1), generating oxidation layer through the oxidization of anode, conducting sealing or a hydrophilic treatment for the oxidation layer, coating sensitization liquid onto this oxidation layer, finally drying and cutting the plates into finished products, wherein back side of the substrate (1) may be covered with a membrane (2) of polymer material after deoiling and cleaning the substrate (1).

## Description

### Field of the Invention

The invention relates to a presensitized plate (PS plate) or Computer-to-Plate plate (CTP plate) with compound support used in the printing industry according to the preamble of claim 1, as well as to a manufacturing process of such plate according to the preamble of claim 4.

### Background of the Invention

Common presensitized plates or CTP plates adopt aluminum support substrate, and have sensitization imaging layer set up on the front side of the substrate. In manufacturing, the surface of the aluminum substrate is roughened, anodized, and conducted sealing or hydrophilic treatment to keep the adsorption of the oxidization layer, and with sensitization imaging layer coated, it is possible to make finished plates. Aluminum substrate has some certain strength and toughness in printing, and is well featured by hydrophilicity and abrasion resistance, etc. as well after roughening and oxidization. However, the utilization quantity of aluminum material is very large, its price has kept rising, and its cost occupies over 75% of that of the plates, so it is urgent to acquire a new kind of plate which could keep the quality and reduce the cost meanwhile. Now, presensitized plates with non-aluminum substrate are also adopted, but they could not replace the presensitized plates with aluminum substrate since their various performance indexes are not reliable or mature.

### Summary of the Invention

Aiming at the deficiency of the existing techniques, it is thus an object of the present invention to provide an offset presensitized plate with compound support which could save aluminum material and enjoys reliable performance, further to provide a manufacturing process of such plate.

A presensitized plate with compound support is proposed, including an aluminum substrate having a front side and a back side, and a sensitization imaging layer set up on the front side of the aluminum substrate, wherein the back side of the substrate is covered with a membrane of polymer materials forming the structure of compound support.

For instance, the substrate may have a thickness of 0,1 to 0,3 mm and the membrane may have a thickness of 0,01 to 0,3 mm.

The membrane could adopt such polymer material with great rigidity as POM, PET, PC or PPS, with the membrane pre-coated with heat-melt adhesive as the prior selection.

Furthermore, a manufacturing process of such plate is proposed, comprising first deoiling and cleaning the aluminum substrate, then conducting electrochemical corrosion and roughening for the surface of the substrate, then generating oxidation layer through the oxidization of anode, then conducting sealing or a hydrophilic treatment for the oxidation layer, then coating sensitization liquid onto this oxidation layer, finally drying and cutting the plates into finished products, wherein back side of the substrate may be covered with a membrane of polymer material after deoiling and cleaning the substrate.

According to the present invention, the step of covering may be performed after any step of the above mentioned process, or even after drying and cutting of plates.

In case the membrane is compounded before the commencement of electrochemical treatment, it is available to keep the back side of aluminum material from contacting the chemicals, save electric energy, avoid over electrochemical reaction at the edges of front side, and enhance the performance of finished products. According to the present invention, it is preferred that the membrane is stuck to and covered on the substrate with heat melting and stitching method.

According to the present invention, it is preferred that the binder for heat melting and stitching adopts ethene - ethylene vinyl acetate copolymer or polymer resin.

The compound support substrate of this invention continues using the advantage of aluminum materials, namely the adsorptive sensitization imaging layer, and sets up membrane layer on the back side. It is possible to use relatively thin aluminum material to keep relatively high quality, greatly reduce the consumption of aluminum, and decrease the cost. The membrane of polymer material is featured by strong toughness; after compounding, the substrate enjoys great tensile strength, so the plate is not easy to break during printing; and also, the polymer material has lower density, which could lighten the weight of finished plates, decrease the requirements on package strength and the transport cost. In addition, polymer membranes have extremely smooth surface, so multiple sheets of presensitized plates overlapped won't scratch the sensitization layer on the front side of each other, and will require no interleaving paper. What's more, the manufacturing process of presensitized plate with compound support is basically accordant with the original one, and the compounding of membrane is simple and quick.

### Brief Description of the Drawings

The invention is described more detailed with reference to the accompanying drawings, in which
- Figure 1: is the schematic diagram of section structure of a presensitized plate, and
- Figure 2: is the schematic diagram of a heat melting and stitching state.

### Detailed Description of the Preferred Embodiment

As shown in the Figures, a substrate 1 has a sensitization imaging layer 3 set up on a front side, and has a membrane 2 of polymer material covered on a back side, which form the structure of compound support. In manufacturing, the aluminum substrate 1 adopted for presensitized plate is 0,142 mm in thickness, the membrane 2 adopts PET pre-coated film of 0,125 mm in thickness; and pre-coating binder adopts ethene - ethylene vinyl acetate copolymer (EVA) or polymer resin.

The manufacturing comprises deoiling and cleaning the aluminum substrate 1, sending it to and between the heat conducting roller and stitching roller of the compound equipment, then covering the membrane 2 to the back side of the substrate 1 by making use of pressure and temperature through heat melting and stitching; then conducting electrochemical corrosion and roughening on the surface of substrate 1, generating oxidation layer through the oxidization of anode on the surface of substrate 1, carrying out sealing treatment for the oxidation layer, and coating sensitization liquid onto this oxidation layer; finally, drying and cutting the plates into finished products.

Relative to presensitized plate with full aluminum substrate, the presensitized plate with compound support obtained has various excellent performances, including weight, fracture resistance, friction safety, and printing adaptability, etc.

In case of manufacturing of a CTP plate, the manufacturing process is basically the same and requires coating image liquid on the substrate 1, and the finished compound support dried and cut enjoys various excellent performances.

## Claims

1. A presensitized plate with compound support, including an aluminum substrate having a front side and a back side, and a sensitization imaging layer set up on the front side of the aluminum substrate, ***characterized* in that** the back side of the substrate (1) is covered with a membrane (2) of polymer material forming the structure of compound support.

2. A presensitized plate according to claim 1, ***characterized* in that** the thickness of the substrate (1) and membrane (2) is 0,1 to 0,3 mm and 0,01 to 0,3 mm respectively.

3. A presensitized plate according to claim 1 or 2, ***characterized* in that** the polymer material adopted for membrane (2) is POM, PET, PC or PPS.

4. A manufacturing process of presensitized plate with compound support according to claim 1, comprising the steps of
- deoiling and cleaning the aluminum substrate (1),
- conducting electrochemical corrosion and roughening for the surface of the substrate (1),
- generating oxidation layer through the oxidization of anode,
- conducting sealing or a hydrophilic treatment for the oxidation layer,
- coating sensitization liquid onto this oxidation layer,
- drying and cutting the plates into finished products, and
***characterized* in** covering the back side of the substrate (1) with a membrane (2) of polymer material after deoiling and cleaning the substrate (1).

5. A process according to claim 4, ***characterized* in** performing the step of covering the membrane (2) on the substrate (1) after any step of the above mentioned process, or even after drying and cutting of the plate.

6. A process according to claim 4 or 5, ***characterized* in that** the membrane (2) is stuck to and covered on the substrate (1) by means of heat melting and stitching.

7. A process according to claim 6, ***characterized* in that** a binder for heat melting and stitching adopts ethene - ethylene vinyl acetate copolymer or polymer resin.
